

## UNITED STATES PATENT OFFICE

HOWARD DIMMIG, OF PORT ARTHUR, TEXAS, ASSIGNOR, BY MESNE ASSIGNMENTS,  
TO THE TEXAS COMPANY, OF NEW YORK, N. Y., A CORPORATION OF DELAWARE

## MANUFACTURE OF LUBRICANTS

No Drawing.

Application filed October 4, 1921. Serial No. 505,318.

This invention relates to the formation of additional normal lead oleate, water and carbon dioxid. The agitation and heating may be continued until there is no free acid present and the lead oleate is then allowed to cool somewhat, for example, to about 200° F., when lubricating oil is added and mixed with the soap to form the desired compound.

I have found that in the production of lubricants containing lead soaps it is desirable to avoid the use of the basic lead salt and employ the normal salt. The basic lead salt,  $2\text{Pb}(\text{C}_{17}\text{H}_{33}\text{COO})_2\text{PbO}$ , is sticky and stringy in character, it is not permanently soluble in hydrocarbon oils, it does not reduce the viscosity of lubricants at low temperatures and is, in fact, wholly unsuited for use in the preparation of lubricating compounds. The normal salt,  $\text{Pb}(\text{C}_{17}\text{H}_{33}\text{COO})_2$ , on the other hand is oily in character, is permanently soluble in oil and reduces the viscosity at low temperatures of the lubricating oil stock with which it is compounded.

In accordance with my invention I react any of the oxids of lead, preferably one of the lower oxids, oleic acid in any suitable form, such as elain or red oil, and carbon dioxid under conditions to form the normal lead salt and then mix the lead soap with a suitable cylinder oil or other lubricating oil to form a homogeneous lubricating compound.

According to my present knowledge and belief, the chemical reactions of the process proceed substantially as follows—



In the preferred manner of carrying on the process the lead oxid and oleic acid are introduced into a mixing kettle and carbon dioxid is blown thru the mixture while heated sufficiently for the reaction. The temperature used varies from about 350° F. to 500° F. If desired mechanical agitating means may be employed, especially during the first stages of the reaction. It is probable that the lead oxid and oleic acid react immediately to form the basic salt. The carbon dioxid then attacks the basic salt with the formation of the normal salt and some lead carbonate, and the oleic acid reacts with the carbonate yielding

The normal soap also possesses the property of reducing the viscosity at low temperatures of the compound into which it enters below that of the oil stock with which it is mixed. The effect of the normal soap on paraffin oils is especially marked, the oleate apparently hindering in some manner the formation of wax crystals. The effect on asphalt base oils is in a less degree but the viscosity of the compound is also reduced at low temperatures below that of the oil stock. The practice of my invention is thus particularly adapted for the production of lubricants adapted for use at cold temperatures.

Various lubricating compounds may be prepared in accordance with my invention, such for example as car oils, driving journal compounds and other lubricants. The proportion of oleate used varies with the type of product desired. For example, summer

car oils require less oleate than winter car oils. The proportion may vary from as low as 2%-10%, which is the proportion ordinarily used for car oils, for instance, to the 5 higher proportions used in the preparation of greases.

Obviously many modifications and variations of the invention, as hereinbefore set forth, may be made without departing from 10 the spirit and scope thereof, and therefore, only such limitations should be imposed as are indicated in the appended claims.

What I claim is:—

- 15 1. The process of manufacturing lubricants which comprises heating a mixture of lead oxid and oleic acid, passing carbon dioxid through the heated ingredients to cause the formation of normal lead oleate and then mixing said oleate with lubricating oil.
- 20 2. The process of manufacturing lubricants which comprises heating a mixture of lead oxid and oleic acid while passing carbon dioxid through the heated mass and then mixing the resulting product with lubricat-25 ing oil.
- 30 3. A lubricant comprising a mineral lubricating oil compounded with normal lead oleate.
- 35 4. A liquid lubricant comprising a mineral lubricating oil compounded with a lead oleate completely and permanently soluble in the oil, and having a viscosity at low temperatures lower than the uncompounded oil.

In witness whereof I have hereunto set my  
35 hand this 26th day of Sept., 1921.

HOWARD DIMMIG.